

Aug. 29, 1967

H. A. READ

3,338,787

VASODILATOR DRUG MIXTURE AND EXCIPIENT THEREFOR

Filed Feb. 24, 1964



HOWARD A. READ  
INVENTOR.

BY Ernest G. Peterson  
AGENT.

# United States Patent Office

3,338,787  
Patented Aug. 29, 1967

1

3,338,787

## VASODILATOR DRUG MIXTURE AND EXCIPIENT THEREFOR

Howard A. Read, Succasunna, N.J., assignor to Hercules Incorporated, a corporation of Delaware  
Filed Feb. 24, 1964, Ser. No. 346,757  
7 Claims. (Cl. 167—82)

This invention relates to an improved form of vasodilator drug mixture which is useful for the preparation of pharmaceutical tablets. More particularly, it relates to a high concentration of pentaerythritol tetranitrate (PETN) as the active therapeutic agent in combination with pentaerythritol as the principal excipient.

The use of PETN as the active therapeutic agent in vasodilators is well known as well as the use of various excipients for reducing the explosive sensitivity of PETN for subsequent processing into pharmaceutical tablets. Conventionally, the tablets are formed by compressing a granulation of the active therapeutic agent in combination with certain inert pharmaceutical excipients. The conventional inert pharmaceutical excipients include such materials as starch, lactose, terra alba, sucrose, dextrose, sorbitol, mannitol, activated clays, any of the well known gums as well as lubricants such as talc, stearic acid, magnesium stearate and in addition, solubilizing agents and the like. These excipients are desirable in preparing a tablet of convenient size and in addition, serve to reduce the concentration of the PETN during preparation of the tablet to minimize any possible hazards which might result through its handling. Generally, under conventional practice, the amount of PETN by weight of the entire mixture has been held to less than 20%. The more recent pharmacopedia, however, is demanding of vasodilator mixtures containing PETN at concentrations

considerably more than 20% by weight. This poses additional problems at these high concentrations for minimizing any possible hazards which might result in preparation of the tablets. The high concentrations of PETN, of course, permit the compounder to prepare tablets of required dosage in a smaller size as well as permit the compounder to add other drugs as desired without excessively increasing the tablet size.

Now, in accordance with the present invention, a vasodilator drug mixture has been developed which, in addition to containing a high concentration of PETN, also has the PETN in finely divided form. Effective oral administration of an organic nitrate therapeutic agent generally requires extremely rapid disintegration of a tablet containing the agent and rapid absorption so that the therapeutic ingredient quickly enters into the blood stream. PETN of extremely fine particle size as encompassed by this invention serves to aid both of the aforementioned requirements.

More specifically, in accordance with the present invention, there is provided a vasodilator drug mixture especially adapted for compounding, the mixture consisting essentially of between 20 and about 35% of PETN having a particle size diameter of not more than 50 microns and between about 65 and about 80% of pentaerythritol having a particle size diameter of not more than 100 microns, all percentages being by weight of the mixture and all ingredients being in intimate mixture, wherein said pentaerythritol is essentially the sole desensitizing excipient or said pentaerythritol and activated clay serve as the desensitizing excipient.

The tests given in the following table demonstrate the desensitizing effect imparted by the excipients of the present invention when utilizing finely divided PETN.

TABLE

|                                                           | Test No.                  |                     |          |          |                     |                   |                   |              |                |                |                |
|-----------------------------------------------------------|---------------------------|---------------------|----------|----------|---------------------|-------------------|-------------------|--------------|----------------|----------------|----------------|
|                                                           | 1                         | 2                   | 3        | 4        | 5                   | 6                 | 7                 | 8            | 9              | 10             | 11             |
| PETN—Type                                                 | Fine                      | Fine                | Fine     | Fine     | Fine                | Fine              | Fine              | Fine         | Fine           | Fine           | Fine           |
| Formula:                                                  |                           |                     |          |          |                     |                   |                   |              |                |                |                |
| PETN, percent                                             | 25.0                      | 25.0                | 25.0     | 25.0     | 25.0                | 30.0              | 32.0              | 35.0         | 35.0           | 35.0           | 35.0           |
| Pentaerythritol, percent                                  | 75.0                      | 67.5                | 67.5     | 68.4     | 68.4                | 63.0              | 59.5              | 58.4         | 58.4           | 58.4           | 58.4           |
| Pharmasorb, percent                                       |                           | 7.5                 | 7.5      | 6.6      | 6.6                 | 7.0               | 8.5               | 6.6          | 6.6            | 6.6            | 6.6            |
| Cap Sensitivity (2" x 8" Ctg.)                            | F-5 gm.<br>S-10 gm.       | F-5 gm.<br>F-20 gm. | F-20 gm. | F-20 gm. | F-5 gm.<br>S-10 gm. | F-Army<br>S-2 gm. | F-Army<br>S-2 gm. | F-#8<br>S-#8 | F-#8<br>S-Army | F-#8<br>S-Army | F-#8<br>S-Army |
| Lead Block Compression (Sixteenth in.):                   |                           |                     |          |          |                     |                   |                   |              |                |                |                |
| 5 gm. initiator                                           | 0                         | 1                   | 1        | 1        | 0                   | 0                 | 0                 | 0            | 20             | 14             | 15             |
| 20 gm. initiator                                          | 1                         | 5                   | 2        | 3        | ½                   | 2                 | 1                 | 2            | 20             | 17             | 17             |
| Detonation Rate 3" x 24" Ctg. Primer (328 gms. Pentolite) | 2 Fail                    | 2 Fail              | 2 Fail   | 2 Fail   | 2 Fail              | 2 Fail            | 2 Fail            | —            | 2,680<br>2,800 | 2,340<br>2,500 | Fail<br>Fail   |
| Particle Size of Pentaerythritol (Diameter in Microns):   | Percent weight—less than— |                     |          |          |                     |                   |                   |              |                |                |                |
| 150                                                       | 100                       | 100                 | 100      | 100      | 100                 | 100               | 100               | 100          | 100            | 100            | 100            |
| 100                                                       | 93                        | 83                  | 96       | 100      | 97                  | 99                | 99                | 99           | 93             | 100            | 100            |
| 75                                                        | 99                        | 80                  | 96       | 99       | 97                  | 99                | 99                | 99           | 80             | 96             | 100            |
| 50                                                        | 95                        | 62                  | 89       | 96       | 87                  | 95                | 95                | 93           | 62             | 89             | 97             |
| 25                                                        | 82                        | 42                  | 65       | 82       | 63                  | 82                | 82                | 77           | 42             | 65             | 84             |
| 10                                                        | 39                        | 22                  | 27       | 40       | 28                  | 39                | 39                | 37           | 22             | 27             | 50             |
| 5                                                         | 7                         | 10                  | 7        | 10       | 7                   | 7                 | 10                | 10           | 7              | 10             | 16             |

F=Failed. S=Shot.

Note.—#6 cap contains approx. 0.25 gm. PETN. #8 cap contains approx. 0.40 gm. PETN. Army cap contains approx. 0.94 gm. PETN. Other caps contain PETN in the amount given.

With reference to the foregoing table, curve A of the appended drawing represents a typical particle size distribution analysis for the "Fine" PETN used in the tests, and curve B represents a typical particle size distribution analysis for pentaerythritol, which gives effective desensitization in accordance with the invention. Here it will be seen that the PETN has a particle size diameter of not more than 50 microns and preferably, not more than about 40 microns; also, that the pentaerythritol has a particle size diameter of not more than 100 microns and preferably approximately as follows: 100% finer than 100 microns, 95% finer than 70 microns, 90-95% finer than 50 microns, 65-85% finer than 25 microns, 25-50% finer than 10 microns, and 5-15% less than 5 microns.

From the foregoing table, it will be seen that a decrease in the particle size of the pentaerythritol gives an improvement in desensitizing effect. For example, Test 2, where the particle size of the pentaerythritol exceeded 100 microns, failed to shoot with a 5 gm. booster cap while Tests 3, 4 and 5, where the particle size did not exceed 100 microns, failed to shoot with the large 20 gm. booster caps. Similarly, Test 9, where the particle size of the pentaerythritol exceeded 100 microns, shot with a #8 electric blasting cap while Tests 8, 10 and 11, where the particle size did not exceed 100 microns, failed to shoot with #8 electric blasting caps.

It will be apparent from the table that several tests have been used for establishing criterion denoting degrees of safety for subsequent processing into pharmaceutical tablets. In one test, the drug mixture is packed into 2" diameter x 8" long paper shells and tested with various sized caps to determine if it will shoot. In another test, the drug mixture is packed into 3" diameter x 24" long fiber tubes and tested for propagation when primed with a 328 grams Pentolite (50/50 PETN/TNT) primer. In still another test, 2 pounds of the drug mixture is poured into a half-gallon paper container. The container is placed on a shock plate which rests on top of a loose-fitting piston which in turn is positioned on a lead cylinder block. A booster cap containing either 5 or 20 grams of PETN is used to prime the charge. After firing the cap, the lead cylinder block is removed, and its length is measured in sixteenths of an inch to determine how much it has been compressed relative to its original length. The amount of compression is expressed as a number representing the number of sixteenths of an inch so measured. The low numbers are indicative of low sensitivity.

The drug mixtures in accordance with the present invention and as used in the tests are compounded by simply intimately mixing the finely divided PETN and the excipient. Within the purview of the invention, the excipient consists essentially of pentaerythritol alone having a particle size of not more than 100 microns or said pentaerythritol with not more than about 15% by weight of particulate highly porous activated clay. Pharmasorb, which is marketed by Minerals and Chemicals Corporation and which was used in the tests, is representative of the latter class of materials and is an additive commonly used in organic nitrate pharmaceutical mixtures. The Pharmasorb used in the tests was "regular" grade and had an average particle size of about 3.8 microns. However, other particulate highly porous activated clays including the heat treated clays are commonly available and suitable for this purpose when used up to about 15% and preferably not more than about 10% by weight of the excipient. The particle size of these clays may range from about 0.01 to about 200 microns, with it being preferred not to exceed about 100 microns in keeping with the desensitizing effect as demonstrated by the maximum particle size diameter for the pentaerythritol.

The ingredients for the drug mixture of this invention may be added separately and intimately mixed, or the excipient first prepared and later mixed with the PETN to form the intimate end product mixture. It will be

appreciated that additional materials such as the gums, lubricants, solubilizing agents and the like heretofore mentioned may be incorporated with the drug mixture of this invention. These additional materials ordinarily will not exceed about 10% by weight of the drug mixture and may be incorporated as an "add" to the mixtures herein described and claimed.

It will be seen, therefore, that this invention may be carried out by the use of various modifications and changes without departing from its spirit and scope, with only such limitations placed thereon as are imposed by the appended claims.

What I claim and desire to protect by Letters Patent is:

1. A vasodilator drug mixture especially adapted for compounding, the mixture consisting essentially of
  - (a) between 20 and about 35% of pentaerythritol tetranitrate having a particle size diameter of not more than 50 microns, and
  - (b) between about 65 and about 80% of pentaerythritol having a particle size diameter of not more than 100 microns.
2. A vasodilator drug mixture especially adapted for compounding, the mixture consisting essentially of
  - (a) between about 25 and about 35% of pentaerythritol tetranitrate having a particle size diameter of not more than about 40 microns,
  - (b) between about 55 and about 70% of pentaerythritol having a particle size diameter of not more than 100 microns, and
  - (c) between about 5 and about 10% of particulate highly porous activated clay, all percentages being by weight of the mixture and all ingredients being in intimate mixture.
3. A vasodilator drug mixture especially adapted for compounding, the mixture consisting essentially of
  - (a) about 25% of pentaerythritol tetranitrate having a particle size diameter of not more than about 40 microns, and
  - (b) about 75% of pentaerythritol having a particle size diameter of not more than 100 microns.
4. A vasodilator drug mixture especially adapted for compounding, the mixture consisting essentially of
  - (a) about 25% of pentaerythritol tetranitrate having a particle size diameter of not more than about 40 microns,
  - (b) about 68% of pentaerythritol having a particle size diameter of not more than 100 microns, and
  - (c) about 7% of particulate highly porous activated clay, all percentages being by weight of the mixture and all ingredients being in intimate mixture.
5. A vasodilator drug mixture especially adapted for compounding, the mixture consisting essentially of
  - (a) about 30% of pentaerythritol tetranitrate having a particle size diameter of not more than about 40 microns,
  - (b) about 63% of pentaerythritol having a particle size diameter of not more than 100 microns, and
  - (c) about 7% of particulate highly porous activated clay, all percentages being by weight of the mixture and all ingredients being in intimate mixture.
6. A vasodilator drug mixture especially adapted for compounding, the mixture consisting essentially of
  - (a) about 35% of pentaerythritol tetranitrate having a particle size diameter of not more than about 40 microns,
  - (b) about 58% of pentaerythritol having a particle size diameter of not more than 100 microns, and
  - (c) about 7% of particulate highly porous activated clay, all percentages being by weight of the mixture and all ingredients being in intimate mixture.
7. An excipient especially adapted for desensitizing a vasodilator drug mixture containing more than 20% of pentaerythritol tetranitrate, the excipient consisting essentially of

- (a) pentaerythritol having a particle size diameter of not more than 100 microns and
- (b) not more than about 15% of particulate highly porous activated clay by weight of the excipient.

## References Cited

## UNITED STATES PATENTS

3,096,242 7/1963 Young ----- 167—65

## OTHER REFERENCES

Berlow et al.: "The Pentaerythritols," Reinhold Publ. Corp., New York, 1958, pages 259, 279-281.  
C & E News, vol. 25, page 1147 (1947).

<sup>5</sup> LEWIS GOTTS, *Primary Examiner.*

ALBERT T. MEYERS, *Examiner.*

G. A. MENTIS, S. K. ROSE, *Assistant Examiners.*